

## UNITED STATES PATENT OFFICE

2,085,002

## ANODIC TREATMENT OF ALUMINUM

Robert W. Buzzard, Kensington, Md.

No Drawing. Application May 22, 1934,  
Serial No. 726,896

4 Claims. (Cl. 204—1)

(Granted under the act of March 3, 1883, as  
amended April 30, 1928; 370 O. G. 757)

This invention relates to a process for forming protective coatings on aluminum or aluminum alloys by using the object to be treated as the anode in a suitable bath.

5 It is the object of this invention to devise a process for the purpose mentioned that will include a considerable range of concentrations of the chemically active component of the bath as well as making it possible to effect the coating 10 over a relatively large range of temperature and voltage conditions.

This application is a continuation in part of my copending application Serial No. 656,761.

The processes for anodic treatment of aluminum in chromic acid solutions heretofore generally used have been restricted to a very definite concentration for the bath, have necessitated a close control of a voltage cycle and also a definite, elevated temperature.

20 In the practice of my invention the article to be treated, after having been thoroughly cleaned, is placed in a bath containing from 4% to 25% of chromic acid. With the article serving as the anode, a constant potential from a source of direct current between 10 volts and 50 volts is applied to the bath, which is kept at a constant temperature between 20° C. and 60° C., for a period of about one hour. Probably the most satisfactory concentration of the chromic acid is 25 9.5%, but it may be varied with good results between the limits above mentioned. Further, it has been found that satisfactory oxide films for definite purposes can be formed in any concentration of chromic acid by properly adjusting the 30 voltage and the temperature. These discoveries 35 are the product of a long and extensive research on the subject. They are neither obvious nor self-evident from previous work on anodic films. The same results cannot be produced by alternating current.

40 A superior film may be formed in a chromic acid bath containing additional chromates, the chromic acid content and the percentage of chromate being varied according to the type of film desired and the particular chromate employed. The temperature and voltage used with this type of bath must be varied to suit the composition of the electrolyte but for any given type of film the voltage is kept constant. As one specific example, there may be mentioned a bath of 5% chromic acid by weight and 5% potassium dichromate by weight using a constant direct current voltage of 40 volts and a constant temperature between 35° C. and 40° C. The film forms 55 rapidly and a satisfactory thickness will be de-

veloped in one-half hour but the corrosion resistant properties are increased if the treatment is continued for an hour.

The film formed by a bath having the composition mentioned in the preceding paragraph is superior in some qualities to those formed in straight chromic acid baths and in general to those formed in straight chromate baths and is not the same type of film as would be obtained from such a treatment in the two baths separately since the chromate acts as a hardener of the film. In fact, the result so obtained is not predictable from a study of the coatings produced in that way. The use of chromic acid and a chromate together is not limited to the particular proportions mentioned as a very good film is formed in a 3% chromic acid bath with 1% of potassium dichromate. The range of concentrations for this compound bath has not been definitely delimited but it is known that satisfactory coatings are formed at most concentrations in which the sum of the percentages of chromic acid and potassium dichromate is not more than 25% of the bath.

As examples of the values of voltages and temperatures that may be used successfully when the concentration of chromic acid is in the neighborhood of 10%, the following may be mentioned: 25 30 volts at 35° C.; 30 volts at 40° C.; 40 volts at 35° C.; 42 volts at 40° C.; 35 volts at 40° C.; 35 volts at 35° C. Or the following cycle may be 30 followed with the temperature held constant between 35° C. and 40° C.: Raise voltage to 40 volts in five minutes, maintain 40 volts for ten minutes, lower to 35 volts in five minutes, maintain 35 35 volts for ten minutes, lower to 30 volts for five minutes and maintain 30 volts for twenty-five minutes. In all cases the voltage referred to is derived from a source of direct current. When the voltage is kept constant at any value, say 40 volts, it may be raised to that value as quickly as 40 the source of power will permit, or as slowly as the operator desires. The duration of treatment depends upon the thickness and type of film desired, the longer times, within limits, producing thicker films. Also, the higher the temperature 45 the softer and darker the film.

It is known that the effect of lowering the temperature of the bath is to reduce the current density, whereas the effect of lowering the voltage is to raise the current density within limits. 50 The effect of increasing the chromic acid concentration at constant voltage and temperature is to increase the current density, but also the effective temperature may be readily lowered with 55

increased chromic acid concentration to counteract this effect.

It has been found in general with the baths described herein that there is one voltage at which a minimum current density is obtained which is namely 40 volts. Raising the voltage or lowering it from this value carries increased current densities. The best corrosion resistance of the film is produced by different temperature, 5 voltage-time cycles in different concentrations. As the concentration of the bath is increased the 10 temperature may first be lowered and then the time-voltage as the concentration increases. It is not recommended that both time and voltage 15 be lower for the same cycle.

It is optional whether the material is washed to remove therefrom the adhering solution, since if such solution is left on it will, under certain conditions, improve the corrosion resistance. 20 Any solution that remains in cracks does not attack the metal or have any detrimental effect and when once the solution is dried on it is very difficult to remove. Commercial application is now being made of this process by the Navy Department 25 and is covered by the Navy specification for the Anodic treatment of aluminum and its alloys.

It is readily apparent that since my bath permits the use of constant voltage and constant 30 temperature it may be used for treating materials both in a continuous process bath and in a batch bath rather than being restricted to batch treatment alone.

The invention described herein may be manufactured and used by or for the Government of

the United States of America for governmental purposes without the payment of any royalty thereon.

I claim:

1. A bath for forming with direct current, by anodic treatment either in batches or in continuous process, protective coatings on articles having aluminum as a constituent, comprising 5% chromic acid and 5% potassium dichromate as a film hardener. 10

2. A bath for forming with direct current, by anodic treatment either in batches or in continuous process, protective coatings on articles having aluminum as a constituent, comprising 3% chromic acid and 1% potassium dichromate 15 as a film hardener.

3. A bath for forming with direct current, by anodic treatment in continuous process, protective coatings on articles having aluminum as a constituent, comprising from 3% to 5% of chromic acid and 1% to 5% of potassium dichromate 20 as a film hardener.

4. A process of forming, with direct current, anodic coatings on material having aluminum as a principal constituent, comprising the steps of 25 utilizing the material to be treated as an anode in a bath containing from 3% to 5% chromic acid and 1% to 5% potassium dichromate as a film hardener, the temperature of said bath being between 35° C and 40° C., and applying to 30 said anode and bath a potential of between 30 volts and 42 volts, the aforesaid steps being applicable as a continuous process.

ROBERT W. BUZZARD.

35